

# United States Patent [19]

Raüm et al.

[11] 3,901,783

[45] Aug. 26, 1975

[54] **METHOD OF PRODUCING SELENIUM CHARGE ELECTROPHOTOGRAPHIC RECORDING PLATES**

[75] Inventors: **Helmut Raüm**, Nurnberg; **John E. Segain**, Gunzenhausen, both of Germany

[73] Assignee: **International Standard Electric Corporation**, New York, N.Y.

[22] Filed: **Feb. 5, 1974**

[21] Appl. No.: **439,807**

[30] **Foreign Application Priority Data**

Feb. 9, 1973 Germany..... 2306332  
Feb. 9, 1973 Germany..... 2306333

[52] U.S. Cl. .... **204/192**

[51] Int. Cl. .... **C23c 15/00**

[58] Field of Search ..... 204/192

[56] **References Cited**

UNITED STATES PATENTS

2,189,580 2/1940 Hewlett..... 204/192

|           |        |                     |         |
|-----------|--------|---------------------|---------|
| 2,903,631 | 9/1959 | Perotte .....       | 204/192 |
| 3,650,737 | 3/1972 | Maissel et al. .... | 204/192 |
| 3,733,258 | 5/1973 | Hanak et al. ....   | 204/192 |

## OTHER PUBLICATIONS

Tanaka, "Photoconductivity of Case Films Prepared by a Vapor Evaporating-Reactive Sputtering Method," Japanese Journal of Applied Physics, Vol. 9, No. 9 (September 1970), pages 1070-1077.

*Primary Examiner*—Oscar R. Vertiz

*Assistant Examiner*—Wayne A. Langel

*Attorney, Agent, or Firm*—John T. O'Halloran;  
Menotti J. Lombardi, Jr.; Vincent Ingrassia

[57]

## ABSTRACT

This relates to a method of producing an electrophotographic recording plate having a non-conducting selenium layer. A small portion of semiconducting material, especially chemical compounds of cadmium, zinc or titanium, is sputtered onto the selenium surface in a glow discharge.

**9 Claims, No Drawings**

**METHOD OF PRODUCING SELENIUM CHARGE  
ELECTROPHOTOGRAPHIC RECORDING PLATES**

**BACKGROUND OF THE INVENTION**

The present invention relates to a process for preparing a selenium charge electrophotographic recording plate with a non-conducting selenium layer arranged on a metal substrate.

In the electrophotographic process there are used recording plates with a conducting substrate on which there is deposited a photoconductive layer of semiconducting material on which a charge pattern is produced by the charge and exposure to light, corresponding to the image pattern. This charge pattern is made visible by the application of a suitable inking powder which, in the course of a further step of the process, is transferred from the recording plate to a sheet of paper where it is fixed. In practice, it has proved particularly suitable to use recording plates employing selenium as the semiconducting material. Certain additives to the selenium improve the electrophotographic properties. The metal substrate on which the selenium layer is deposited, consists either of a rigid metal plate or of a metal cylinder, or else of a flexible metal foil, such as a steel tape. Onto this metal substrate the selenium is usually deposited by way of evaporation under vacuum.

The known electrophotographic recording plates with a selenium layer still have certain disadvantages. First, it is impossible for larger black areas to be reproduced as such, because the charge on the selenium layer is chiefly positioned in the marginal areas of the thus imaged surfaces.

Second, only pure black-and-white patterns can be reduced satisfactorily, whereas patterns with medium shades yield poor reproduction. There has been an attempt to overcome this disadvantage by using optical rasters during the imaging and disintegrating the image into a great number of individual image spots (points). However, this disintegration is unwanted in many cases, especially in the reproduction of photographs. Further, this does not substantially increase the gray scales to be reproduced.

**SUMMARY OF THE INVENTION**

It is the object of the present invention to provide a process of preparing electrophotographic recording plates with a non-conducting selenium layer which permits reproduction of larger black areas, and with the aid of which it is possible to reproduce a greater number of different gray scales.

According to a broad aspect of the invention, there is provided a method of preparing a selenium charge electrophotographic recording plate having a selenium layer deposited on a metal substrate comprising the steps of depositing selenium on a metal substrate by evaporation under vacuum to form a selenium layer, depositing a thin coating of a semiconducting material on a metal plate, subjecting the selenium coated metal substrate and said metal plate having a semiconducting material thereon to a glow discharge whereby a portion of said semiconducting material is deposited on said selenium layer.

Although the deposited amounts of semiconducting substance are extremely small, there is achieved a substantial improvement in the recording plates, permitting the reproduction of larger black areas as well as a

great number of gray scales with the aid of such recording plates.

The aforementioned advantages will only be achieved when the application is effected in the course of a glow discharge. The glow discharge itself also has an influence upon the improvement in the electrophotographic reproducibility of the selenium layer.

The above and other objects of the present invention will be more clearly understood from the following detailed description.

**DESCRIPTION OF THE PREFERRED  
EMBODIMENT**

The application of the semiconducting substance is effected in such a way that a metal plate provided with a coating of the semiconducting substance to be used, is arranged as the cathode in a glow discharge, while the anode is formed by the selenium layer of the recording plate. Both the cathode and the anode are arranged at a certain distance apart each other in a suitable gas atmosphere. As gases for the glow discharge, it has proved particularly suitable to use inert gases, such as nitrogen or rare gases.

A further improvement in the reproducibility of the selenium layers can be obtained in that the metal plate used as the cathode, is provided on its surface facing the selenium surface, with a pattern of recesses. These recesses may also extend entirely through the metal plate forming the cathode, so that the cathode is a perforated metal plate.

The glow discharge is preferably carried out under a pressure in the order of  $10^{-1}$  to  $10^{-2}$  torr (mm Hg). In the course of this, there is used a voltage in the order of 800 to 2,000 V, with the current flow amounting to values between 20 and 200 milliamperes. The selenium surface is exposed to this glow discharge for a period of time ranging between half a minute and sixty minutes. Preferably, an inert gas is used for the glow discharge, hence a gas which, under the glow-discharge conditions does not chemically combine with either the substrate material or the selenium. As a suitable inert gas, it is possible to use e.g. nitrogen or else a rare gas, such as argon.

Surprisingly, oxygen may be used as the gas for the glow discharge. Oxygen, of course, reacts with the selenium, but this reaction has no influence upon the desired effect. No disadvantageous effects upon the electrophotographic properties of the selenium have been noticed when using oxygen.

Suitable semiconducting materials for depositing onto the selenium surface are, in particular, semiconducting cadmium compounds, semiconducting zinc compounds and semiconducting titanium oxide.

Of the semiconducting cadmium compounds, cadmium sulfide and cadmium selenide are particularly suitable.

Of the semiconducting zinc compounds, zinc oxide and zinc sulfide are particularly suitable.

In the case of rigid plates, it has proved particularly suitable to use polished aluminum as the metallic substrate while in the case of flexible foils, polished steel tapes are preferably used.

Onto the completely smooth and well-cleaned metal substrate, the selenium is deposited by way of evaporation under vacuum in the form of a layer in the order of 10 to 100 microns thick. For improving its electrophotographic properties, the selenium may still be pro-

vided with small additions. Thus, for example, it is of advantage to use an addition of 0.5 per cent by weight of arsenic in order to prevent a later crystallization of the selenium layer. In cases where the recording plates are intended to be exposed to X-rays, it has proved particularly suitable to provide additions of metals with a high atomic weight, or compounds of such metals. Lead or lead compounds are especially suitable for this purpose.

The selenium-coated substrate is placed at a suitable distance from a metal plate provided with a thin coating of the semiconducting material to be deposited, in an inert gas atmosphere under a pressure of  $10^{-1}$  to  $10^{-2}$  torr, and a voltage is applied ranging between 800 and 2000 V. The metal plate provided with the layer of semiconducting substance to be deposited forms the cathode while the selenium layer forms the anode. During glow discharge, there will flow a current ranging between 20 and 200 milliamperes. Action lasts for a period ranging between half a minute and sixty minutes.

The resulting electrophotographic recording plates show substantially improved reproducibility, especially of larger black areas, and permit reproduction of a large number of gray scales.

It is to be understood that the foregoing description of specific examples of this invention is made by way of example only and is not to be considered as a limitation on its scope.

As a further means of obtaining the desired increase in the number of gray scales reproducible, the surface of a selenium layer is subjected as the cathode to the glow discharge. A polished plate of aluminum is preferably used as the anode. Glow discharge is carried out under the above described conditions causing a great number of slight imperfections in the selenium surface during glow discharge. The imperfections are uniformly distributed over the entire selenium surface, however, the disintegration of the image into individual spots does not occur as is the case when using an optical raster.

We claim:

1. A method of preparing a selenium charge electro-photographic recording plate having a selenium layer

5 deposited on a metal substrate comprising the steps of: depositing selenium on a metal substrate by evaporation under vacuum to form a selenium layer; depositing a thin coating of a semiconducting material selected from the group consisting of cadmium sulfide, zinc oxide and zinc sulfide on a metal plate; thereafter sputtering a portion of said semiconducting material on said selenium layer by subjecting the selenium coated metal substrate and said metal plate to a glow discharge.

2. A method of preparing a selenium charge electro-photographic recording plate according to claim 1, wherein said glow discharge is carried out under a pressure within the range of  $10^{-1}$  to  $10^{-2}$  torr at a voltage within the range of 800 to 2,000 volts.

3. A method of preparing a selenium charge electro-photographic recording plate according to claim 2, wherein said glow discharge is carried out for a period of time ranging between 30 seconds to 60 minutes.

4. A method of preparing a selenium charge electro-photographic recording plate according to claim 1, wherein said metal plate has a pattern of recesses thereon.

5. A method of preparing a selenium charge electro-photographic recording plate according to claim 1, wherein said metal plate used as the cathode is a perforated metal plate.

6. A method of preparing a selenium charge electro-photographic recording plate according to claim 1, wherein said glow discharge is carried out in an inert gas atmosphere.

7. A method of preparing a selenium charge electro-photographic recording plate according to claim 1, wherein said glow discharge is carried out in nitrogen.

8. A method of preparing a selenium charge electro-photographic recording plate according to claim 1, wherein said glow discharge is carried out in oxygen.

9. A method of preparing a selenium charge electro-photographic recording plate according to claim 1, wherein said metal plate is a polished plate of aluminum.

\* \* \* \* \*